

## UNITED STATES PATENT OFFICE

2,321,775

## DRY CARROTING FUR

Jack D. Sartakoff, Douglaston, Long Island, N. Y.,  
assignor to No-Mercury Felt Corporation, a corporation of New York

No Drawing. Application June 2, 1942,  
Serial No. 445,454

8 Claims. (Cl. 8—112)

This invention relates to the treatment of fur in its preparation for the manufacture of felt hats and is particularly directed to that step which has to do with the carroting of the fur to render it feltable. This application is a continuation-in-part of parent application, Serial No. 405,645, filed August 6, 1941.

In order that the invention may be clearly understood, it is desirable to explain the manner in which furs have heretofore been treated to prepare them for carroting and the subsequent carroting thereof.

It has been the universal practice to deliver pelts to the carroting establishment in the condition in which they are stripped from the carcass, i. e., with the flesh side out. To prepare them for carroting, these pelts, which are generally quite dry, are first placed in a tumbling barrel containing sawdust wet with water. They are tumbled in this barrel with the sawdust for a sufficient period to clean the dirt and flesh from the pelts and incidentally soften the pelts so that they become sufficiently pliable to be readily handled. This tumbling operation with sawdust in the presence of water is purely a cleaning operation. It forms no part of the carroting operation.

At the conclusion of this cleaning operation, the pelts are slit and opened and they are thereupon trimmed to cut off ears, paws, tails, and other undesirable parts, and they may be then clipped or pulled to remove the hard, horny ends of the individual long hairs which are sometimes called the water hairs.

Thereafter it is the practice to stack the pelts flat, generally skin to skin and fur to fur, and place them in storage, where they are permitted to lose most of the cleaning water. In this condition, the pelts are very flexible and remain so until they are withdrawn from the stack for the carroting operation.

Isolated attempts have been made to carrot fur by mechanical brushing or spray operation, but these have for various reasons not come into general use. The carroting operation has long been universally carried out by laying the pelts flat with the fur side up, upon a suitable table, and applying a so-called carroting solution to the fur, by means of a brush in the hand of a skilled operative. Through the years a wide variety of carroting solutions have been employed. By far the most common is the so-called mercury nitrate carrot which has been used sometimes alone and sometimes with other included constituents, such as oxidizing agents.

Nitric and sulphuric acid carrots have also been employed, as well as solutions embodying the permanganates, chloric acid, etc. It is not necessary here to specify all of these carroting solutions for they are well known in the art. Suffice it here to point out that, when a carrot is applied by a brush, as stated, the carroting solution has always been of a dilute character. Those skilled in the art have avoided the use of strong active carrots for it has been universally recognized that overcarroting, such as results from brush application of too strong a carrot, is highly detrimental to the fur. Furthermore strong solutions are dangerous to the user, and brushes, rubber gloves and other application equipment will withstand only relatively weak dilute carrots. Consequently the carrots which have been used since the beginning of the art have invariably been dilute aqueous solutions.

When attempt is made to brush furs with such solutions, it is recognized that appreciable amounts of such solution of the carrot must be applied to the fur, for, as the brush passes over the fur, it tends to flatten down the fur fibers and, unless the fur is practically soaked, only a relatively small portion of the length of the fibers are wet with the carrot, leaving the base portion of the fibers substantially untreated. Brush application, under ordinary working conditions, cannot produce uniform treatment throughout the length of the fur fibers and some fibers invariably will be overcarroted while others will be deficient in the carroting solution. Brush carroted fur leaves the brushing operation in wet matted condition.

These wet carroted pelts are sometimes piled for a day or more to permit the carrot to react. They are thereafter spread for drying, which is sometimes carried out at atmospheric temperature for about one or two days. Otherwise artificial drying is employed, in which case the pelts may be heated to temperatures varying from 100° to 220° F., for a period of between one and two hours. After they are dried, the flesh side is moistened (i. e. "wet down") and they are then piled under burlap until such time as it is desired to cut the fur from the skin.

The fur side of the pelt is then thoroughly brushed, so as to free the fur fibers from the matting which is invariably present to some degree. This brushing tends to separate the individual fur fibers, but very often is accompanied by material waste of the fur which it is necessary to brush or tear out in order to eliminate the matting. After the pelts have been brushed,

they are sorted and counted and bundled for cutting and they thereupon go to the cutting operation where the fur fibers are removed from the skin. The fur is subsequently blown and subjected to other operations preparatory to actually felting it into hat bodies.

The foregoing carroting practice, which has been common in this art for decades, may be summarized as embodying the following steps:

- I. Apply carroting solution
- II. Pile for a period to permit the carrot to react
- III. Spread for drying
- IV. Dry
- V. Wet down
- VI. Pile under burlap until pliable
- VII. Brush to eliminate matting which has occurred
- VIII. Sort, count and bundle for cutting

These steps are the steps from carroting to cutting. Several of them must be carried out by highly skilled operatives and all of them require repeated handling of the pelts, with incident time consuming operations extending over protracted periods. These operations are expensive and any step or steps which it is possible to eliminate, will cheapen the cost of preparing furs for felting. These facts have been recognized for many years, but, although many have tried to evolve simpler and cheaper methods, no satisfactory commercial way of solving the problem has been discovered by anyone. Consequentially, the practice which I have above enumerated continues to be, aside from the present invention, practically the only method in use to this day.

One of the most pronounced drawbacks in the accepted method of carroting pelts is the fact that the carroting operation wets the pelt with a carrot which must be relatively dilute for the reasons given. This sometimes requires piling so that the carrot may be given sufficient time to react. In all cases it requires prolonged drying so that the fur may be brushed and it requires brushing, for after a pelt has been wet according to brush carroting practice, the matting is frequently so severe that it can only be removed in this manner.

From prolonged study of the problem, I concluded that, if it were possible to eliminate this wetting of the pelt by a carroting solution, many of the steps heretofore necessary would be eliminated and I therefore sought some appropriate method of carroting without this wetting of the pelts.

I am aware that attempts have been made to carrot by the use of appropriate gases, but these attempts have not proven practical. I am also aware of United States Patent No. 339,349, issued April 6, 1886, to Edmund Tweedy, Henry L. Brevoort and Isaiah L. Roberts on the process of preparing fur for felting. According to that patent, pelts are placed in a tumbling barrel with such dusty substances as powdered silica and powdered air slaked lime, chalk, fuller's earth or potter's clay, together with a relatively small quantity of marbles, pebbles or iron balls and are tumbled for a period of say eight hours. Although this patent has been known to the art for over half a century, the process described in this patent has never gone into practical use so far as I am aware and it has not solved the problem which, during the long intervening period, continued to vex this industry.

According to the Tweedy et al patent, the pur-

pose of the powdered silica is to abrade off the coating of the fur fibers, while the slaked lime, fuller's earth, powdered chalk or potter's clay serve to absorb the grease which coats the individual fur fibers. The marbles, pebbles or iron balls are used in a quantity of one-fourth

of the bulk of the mass and their purpose is to beat the powdered material against the coating on the fibers. The patent states that a rapid movement of the tumbling receptacle will produce the required effect quicker than a slow one provided that the movement is not so rapid that the particles will be held against the sides of the receptacle by centrifugal force.

I have carried out a very large number of experiments and tests utilizing a tumbling drum and these tests have very conclusively shown the reason why the process set forth in the Tweedy et al. patent did not and could not possibly solve the problem confronting the art prior to the advent of the present invention.

For example, a number of tests were carried out wherein English rack pelts (sometimes referred to as Scotch cony) were placed in a tumbling drum in dry condition with crushed abrasive material, such as powdered silica, of less bulk than the pelts. The drum was rotated to tumble the pelts and silica together at various speeds for various periods ranging up to several hours. These tests conclusively showed that where such abrasive material was tumbled with the pelts for even a period of an hour or two, the pelts were badly cut and damaged and appreciable quantities of the fur fibers were abraded away and made unfit for use. The loss of fur was so great as to render the operation wholly uncommercial. Since powdered abrasive alone so destroys the pelts as to render the operation uncommercial, it is manifest that the addition of iron balls or pebbles to beat the abrasive against the fibers would produce an even worse condition and if this operation were carried out for eight hours, the results would be disastrous from a commercial aspect. Moreover, the powdered materials present are substantially chemically inert and are obviously intended by the patentees merely to soak up the grease. They exert no carroting action.

I have also carried out tests wherein pelts were tumbled in a drum with crushed abrasive and relatively small quantities of well known dilute commercial carrots. These tests demonstrated that, unless a sufficient amount of these commercial carrots were used as to provide a very considerable free flowing liquid in the drum, no satisfactory commercial felt could be obtained. Unless there were enough liquid present to practically soak the fur, the tumbling had to be so protracted that the loss or waste of fur, due to abrasion, rendered the operation wholly uncommercial.

As a result of the very large number of tests carried out under the most careful and painstaking control, I have discovered that it is possible to effectually and commercially carrot pelts without undue waste of fur and in substantially dry condition by tumbling such pelts in a tumbling drum with pieces of an appropriate attrition material or materials, in the presence of a carroting solution of appreciably greater strength than could possibly be used for brush application and in such quantities that, in cooperation with the attrition material, the fur will be effectually carotted within an astonishingly short period of

time and will be substantially dry at the conclusion of the operation.

I have discovered that through the conjoint use of an attrition material and such a strong, highly active carroting solution, I am able to obtain the necessary carroting action, when using such small quantities of the carrot that it may be carried upon pieces of attrition material without leaving free liquid in the drum. The highly active carroting solution appears to be adsorbed in an imperceptible highly active layer on the surface of the attrition material, ready to act on the fur. Thorough tests, substantiated by actual commercial production of hats, have demonstrated that the pelts so treated do not require protracted drying and that in lieu of the eight steps which I have hereinbefore enumerated as common to general present day practice, I am able to produce a superior product with less waste and in but three steps and with appreciable saving of carroting chemicals. The method by which this is accomplished constitutes the present invention.

According to the present invention, carroting may be effected by a strong, active carroting solution, even with concentrated nitric and concentrated sulphuric acids, either alone or with other chemicals. This is made possible by effecting the carroting by means of solid attrition material carrying the chemically active carrot, thus avoiding the dangers inherent in handling corrosive liquids and also ensuring that the carroting agent is evenly distributed, instead of tending to segregate in various areas as more or less scattered and separated pools, which leave insufficient carroting agent in other areas.

Sufficient attrition material is present to ensure that it rubs, in tumbling, freely and repeatedly over every part of the fur on the skins present. For this purpose it usually seems best to tumble with somewhere nearly equal bulks of skins and attrition material, that is, somewhere nearly equal weights if the skins and material have about the same specific gravity.

In practically carrying out this invention, I place in a tumbling drum pieces of an attrition material, hereinafter more specifically described, together with the pelts to be carotted and a relatively small quantity of a strong, active carroting solution. The drum is rotated to drum tumble the contents for a relatively short period (fifteen or thirty minutes will generally suffice). Thereafter I discharge the contents of the drum into a suitable foraminous cage which is rotated for a sufficient period to cage tumble the pelts and thus separate out the attrition material through the foramina in the cage. While the pelts are being caged, they are preferably subjected to moving heated air, so that, during the few minutes which it is necessary to separate out the attrition material, the pelts are ventilated and aired. The pelts are taken from the cage in carotted condition with the fur in fine, open, fluffy condition and they may be passed directly to the cutting knives and the fur thus cut from the skins. I do not have to pile for a period to permit the carrot to react. I do not have to dry over protracted periods. I do not have to brush. I save at least half a dozen handlings of the pelts and I obtain good felts.

Some of the tests which I have carried out will now be described in some detail, together with certain observations which will assist those skilled in the art in the practising of the present invention.

#### Example 1

5 5600 grams of powdered flint, 80 mesh were wet with 100 cc. of water and introduced into the drum with the addition of 100 cc. of concentrated sulphuric acid. The drum was rotated until the abrasive and the acid were thoroughly mixed.

10 It was found that the small amount of acid used coated the abrasive, so that the abrasive was, to all appearances, substantially dry, although the acid was adsorbed on its surface.

15 Into the drum was then introduced 25 English racks weighing 1400 grams and the drum was thereupon rotated for 60 minutes. The skins were then removed, the fur was cut and blown. From this fur thoroughly satisfactory commercial felts were made. It was found however that too much fur had been abraded away and lost to render this procedure practical, particularly because of prevailing high prices of the raw fur.

#### Example 2

20 4000 grams of the same 80 mesh powdered flint were introduced into the drum with 100 cc. of concentrated nitric acid and 50 cc. of concentrated sulphuric acid. This made a strong acid carrot. The drum was rotated until the acid and abrasive were thoroughly mixed, at which time it was found that, to all appearances, the abrasive was substantially dry.

25 30 Into the drum was then introduced 25 English racks weighing 1300 grams and the drum was rotated for 65 minutes. The treated skins were cut and tested and showed satisfactory shrinkage and good felts. The fur used in this test exhibited the phenomenon of yellow carroting. Here again there was considerable loss of fur due to abrasion.

35 40 In carrying out tests of the invention wherein the fur was subjected to attrition, in the presence of an acid, various acids in various amounts were used. Where it was found that the acid was present in such amounts that it might tend to deteriorate the fur, this acid condition was partially neutralized to render the fur less acid before the fur was removed from the drum. I accomplished this result in various tests by introducing into the drum appropriate quantities of neutralizing salts like ammonium carbonate, and sodium carbonate or alkalis such as caustic 45 soda, or the like, and then rotating the drum for a while, until the acid character of the fur had been lessened to the point desired. I found this method of treatment very convenient and satisfactory for the control of acidity.

#### Example 3

55 4000 grams of 80 mesh abrasive, wet with 100 cc. of water, were introduced into the drum with 100 cc. concentrated nitric acid and 50 cc. concentrated sulphuric acid, making a strong acid carrot, and the drum was rotated until the contents were thoroughly mixed. There was then introduced into the drum 25 English racks weighing 1300 grams and the drum was then rotated for 60 minutes.

60 65 There were then introduced into the drum 1000 additional grams of abrasive with which had been thoroughly admixed 50 grams of pulverized potassium permanganate. The drum was then 70 closed and rotation was continued of the whole mass for 30 minutes longer. The fur thus treated was subsequently tested and found to be entirely satisfactory and the resulting felt commercial.

75 The potassium permanganate which was introduced functioned as an oxidizer. In lieu of the

potassium permanganate thus employed, I have found that other per salts, such as ammonium persulfate  $(\text{NH}_4)_2\text{S}_2\text{O}_8$  or potassium persulfate, or any other appropriate oxidizer, such as hydrogen peroxide are useful.

I have also substituted a strong solution of sulfamic acid  $(\text{NH}_2\text{SO}_3\text{H})$  for the other acids and have found that it gives good results.

In all of the tests, wherein I used silica or some other abrasive material as a carrier for the carrot in the drum, I found that the abrasive action on the fur caused a considerable waste of fur fiber. In practice I may use such an abrasive as flint, pumice, carborundum or some other similar abrasive and while satisfactory felts may be obtained by combining this type of material and a strong highly active carrot, I have found it better and more economical to employ an attrition material which is not generally classed as an abrasive.

For example: I tried comminuted rubber as a carrier and found that the waste of fur was negligible but difficulty was experienced in separating the rubber particles from the fur after the carroting operation. I then tried shredded rubber which was obtained by shredding tire inner tubes into strips about 1 inch long and  $\frac{1}{8}$  to  $\frac{1}{4}$  of an inch wide. Several tests, as well as commercial production, were carried out with this latter material. Note the following:

#### Example 4

24 lbs. of shredded rubber were placed in the factory drum and to this was added a mixture of 800 cc. nitric acid mixed with 640 cc. of the peroxide to produce a strong carrot. Then there were placed in the drum 200 skins of English racks, approximating 26 lbs. and tumbled for 15 minutes, and the rubber separated from the skins.

Very satisfactory commercial felts resulted from fur carroted by this procedure and the waste was negligible.

#### Example 5

In the drum, 1500 grams of shredded rubber were charged with 300 cc. of a 15° Bé. mixture of chloric and sulphuric acids to form a strong carrot. 24 flat English racks weighing 1320 grams were introduced and tumbled for 30 minutes and then removed from the drum and the rubber and the skins separated. Very satisfactory felts were made from this fur.

Up to about the time when I conducted the tests which used rubber as the carrier, I had employed an unlined wooden tumbling drum. I found that this drum soaked up considerable acid so that accurate computation of the acid for controlled carroting was difficult. Moreover the wood deteriorated under the action of the strong carroting solutions. I therefore lined the drum with glass and was thereafter better able to compute the amounts of carrot used. The drum structure employed was a twelve sided drum of approximately 42" diameter with flat ends and mounted to rotate with its axis horizontal and it was driven at approximately 17 R. P. M. It had one interior baffle extending longitudinally and projecting inwardly several inches from a removable charging and discharging door in its periphery. It was originally unlined but later lined with glass.

In addition to rubber, I tried many other non-abrasive materials as carrying agents for the carroting solution. Sawdust did not prove satisfactory for it withheld too much of the solution

and with a strong nitric acid carrot there was too much danger of fire. Wooden chips, suitably pretreated to render them non-absorbent and practically inert, were used to produce satisfactory results. Note the following:

#### Example 6

1020 grams of wooden chips in the form of match sticks which had been boiled in paraffin wax and cooled, were introduced into the drum and then there was added 100 cc. of nitric acid and 80 cc. of hydrogen peroxide (concentrated) to produce a strong carrot. 24 English racks weighing 1580 grams were introduced and tumbled for approximately 20 minutes. Tested subsequently in the laboratory they yielded very satisfactory felts.

Here also the waste of fur was negligible.

This and further tests showed that it was highly desirable for the best commercial results to use as the carrier an attrition material which would be substantially inert to the strong carrots used in connection therewith. This is not strictly chemically true of rubber which reacts slowly and in due time will deteriorate. Thus while it is possible to use rubber or similar attrition materials which are for practical purposes substantially inert, I prefer, as the best practice, to use a more inert material, so that it can be used over and over again without being changed and with substantially constant results which are conducive to controlled carroting, i. e., carroting which can be carried out in successive batches with uniform and computable results.

I have found that certain natural or synthetic resins and plastics are very well adapted for this use. For example, highly satisfactory ends have been obtained through the employment of natural and synthetic resins and plastics, such as solidified vinyl resins, "Lucite," "Polystyrene," bituminous materials, asphalt, etc., which are water-resistant, acid-resistant, and caustic-resistant to a high degree. Materials possessing these characteristics are well adapted for employment with all the ingredients used in present-day carrots, even when such carrots are employed in very strong active condition. Note the following:

#### Example 7

32 pounds of the synthetic resin "Polystyrene," in pieces of a size to pass a  $\frac{3}{8}$ " mesh screen and free from dust, were used in the glass lined drum with a prepared mixture of 600 cc. nitric acid (39-40° Bé.) and 512 cc. of 100 volume hydrogen peroxide. This is a strong highly active carrot. The drum was rotated until the solution had been distributed over the resin particles and there was then introduced into the drum 200 English racks, weighing 29 pounds, 2 ounces. The whole was then drum tumbled for 15 minutes. The drum was then inverted and the contents dumped into a foraminous cage mounted to rotate on a horizontal axis. The felts were tumbled in this rotating cage for 15 minutes, i. e., cage tumbled, at room temperature. They were then spread on the floor for about one hour and then bundled until the next day when they were cut. Very good felts resulted from this procedure and there was a negligible waste of fur.

#### Example 8

In Example 7, above given, the synthetic resin carrier was fresh material which had not been used before. It was found that, after use, some of the acid constituents of the carroting solution

adhered to the carrier in a more or less permanent fashion, i. e., up to a more or less constant degree. Consequently, when the technique and performance of Example 7 was repeated, using again the same carrier as used in Example 7, it was found, by titration, that approximately 14% of the acid was retained on the synthetic resin. Consequently in repeating this example under identical conditions adhered to in Example 7, it was only necessary to add 86% as much acid as in Example 7. With subsequent batches of fur, re-using the same synthetic resin, it was found that the adhesion of the acid remained substantially constant at approximately 14% and this was taken in account in the adding of the carrottting solution to be used in conjunction therewith.

From my investigations it would appear that I may employ other forms of resins or other materials which are relatively hard and suitably non-reactive to the carrottting solutions employed. Tests have indicated that I may use particles of hard paraffin wax as a carrying medium for the carrot and that I may also employ relatively hard asphalt particles, either in natural state or after hardening them with sulphur. The advantage of these materials, as well as resinous materials is that they do not tend to stick to the carrottted fur and can be readily disassociated therefrom before cutting the fur from the skin. Moreover, they are substantially inert and non-reactive with the strong carrots employed. I have obtained the best results from pieces which pass the  $\frac{3}{8}$ " mesh screen but eliminating the smallest sizes and dust.

In Example 7 I have referred to cage tumbling of the pelts at atmospheric temperature and of subsequently laying them on the floor for an hour. In the carrottting of furs according to this invention an appreciable portion of the carrot is rubbed off of the carrier material on to the fur fibers as the carrier rubs over the fur. Consequently at the conclusion of the carrottting operation of tumbling, the fur fibers may be slightly damp, although the fur is never actually wet. It is because of this phenomenon that my process has become known in the trade as dry carrottting. However, some moisture may be present at the conclusion of the drum tumbling operation and it was to permit the loss of some of this moisture that the fur was laid on the floor to ventilate for an hour before bundling.

According to the present invention, however, even this short period of ventilation and this accompanying handling of the pelts may be omitted by circulating through the cage, during the cage tumbling thereof, a current of heated air. When this is done, it is found that the pelts come out of the caging operation dry enough to be immediately stacked, with the fur in a fine fluffy condition and entirely free from any matting tendency, so that they can go to the cutting machine immediately if desired.

Another discovery which I have made, and which is of great importance from a practical standpoint has to do with the preparation of the pelts for the carrottting operation. For example I found by experimentation that, when the pelts were introduced into the drum with the flesh side of the pelt uncovered, it required much more carrottting solution to properly carrott them, than is the case if the flesh side of the pelt were covered or otherwise protected against contact with the carrot or with the attrition material. This I have found, is due to the fact that, when

the flesh side of the pelt is exposed, a considerable portion of the carrottting solution is wasted by acting upon this side of the pelt where it does no good. In fact it does harm for, in conjunction with the attrition material, particularly where an abrasive is used, the thinner portions of the skin may be so tenderized that subsequent cutting of the skin involves considerable loss of fur.

I made the discovery that, if the flesh side of the skin were protected against the action of the strong carrot and the attrition material, I not only materially economize in the amount of carrot required, but I also leave the skin in perfect condition for subsequent cutting.

When the flesh side of the skin is protected from the action of the carrottting solution, I have found that the amount of carrottting solution needed is almost directly proportional to the weight of fur on the skin, thus making it possible to predict in advance the amount of solution needed and eliminating any need for depending on the judgment of the carrottting workman in treating the skins of different lots.

This protection of the skin can be accomplished by covering the flesh side of the pelt in various ways. For instance I may coat the flesh side of the skin prior to carrottting with an appropriate coating material, e. g., a nitrocellulose lacquer, or I may secure skins in pairs to one another flesh side to flesh side. However, I have found the most convenient practice is to fold the individual skins longitudinally so that the two lateral halves of each pelt mutually cover each other in substantially face abutting relation, flesh side to flesh side. This leaves only the fur side exposed to the carrottting action during tumbling and brings about remarkable economy and the advantages to which I have referred. This folding of the pelts does not add any appreciable labor. It simply means that, after the skins have come out of the cleaning operation in moist pliable condition, they are folded transversely as they are stacked to await the carrottting operation. The folded condition of the skin is natural to the skin wherein the fur grows on the outside and consequently the pelt will readily retain this condition if it is stacked in this shape at the conclusion of the appropriate cleaning operation.

An example of highly satisfactory commercial procedure in this connection is as follows:

#### Example 9

6½ lbs. of pieces of substantially inert synthetic resin (dust free) were introduced into the drum with 125 cc. of nitric acid, 38° Bé., 125 cc. hydrogen peroxide 13° Bé. (100 volume), 6 grams zinc sulphate, and 3 grams of chromium potassium alum. This is strong carrot. The drum was revolved for a time to thoroughly admix the carrottting solution and to deposit it in a thin, substantially imperceptible, layer over the pieces of resin. There were then placed in the drum 50 folded English racks weighing 6½ pounds. The drum was then rotated to drum tumble the pelts for 15 minutes.

At the conclusion of this operation, the skins were dumped from the drum into the foraminous cage which was contained within a housing through which air heated to approximately 140° F. was moving. They were cage tumbled for 15 minutes, during which time all of the resin was freed from the pelts. The cage was then opened and the pelts removed. They were found to be to all appearances perfectly dry.

The fur was particularly fluffy. There was not the slightest sign of matting and these skins were ready to be cut. The waste from this operation was so meagre that there was not enough waste fur to cover the palm of the hand. When cut and felted, they produced highly satisfactory felts and it is to be noted that in this entire operation the skins were not touched by the human hand from the time they started the carroting operation until the time that they were removed to be sent to the cutting machine. Such a procedure is revolutionary in the carroting art. Nothing before has even distantly approached its efficiency or economy.

It will be noted that in the last example, there is included, zinc sulphate and chromium potassium alum in very small quantities. These appear to act like catalysts while the latter in particular appears to react with the keratin of the pelt, so as to have a slight tanning action thereon which makes the handling of the pelt easier during the cutting operation.

I have not attempted by any means to enumerate all of the tests which have been made with respect to the present invention. They have conclusively shown that, through the employment of this invention, furs may be carotted without undue waste and in a highly economical and commercial manner.

I have referred mainly to the use of carrots embodying acid alone and with hydrogen peroxide and other agents. Instead of using peroxide I may use a permanganate carrot or numerous other types of carrots which are used generally in dilute form in the art for brush carroting.

#### Example 10

350 cc. of potassium permanganate (6.2% solution) and 50 cc. of commercial concentrated sulphuric acid were placed in a drum with 9 pounds of pieces of synthetic resin and after being thoroughly distributed, 50 folded English racks weighing 6 pounds 4 ounces were introduced. The drum was rotated for 15 minutes thereafter and the carotted pelts were caged for 15 minutes at room temperature. Very satisfactory felts were obtained.

I have found that I can satisfactorily use practically every carroting chemical or chemicals that have been employed for brush application, but with this difference, namely, that, whereas the brush application employs a very dilute solution or weak carrot, I can employ a carroting solution so strong that it could not possibly be used for brush carroting and I find such a strong, highly active carrot is conducive to the highest efficiency in dry carroting according to this invention. For example, I have found it useful to employ solutions two or three times as strong as could possibly be employed for brush application. Thus, if a particular solution for brush application would run about 10° Bé., the corresponding solution which I have used, ran at least twice, or better three times, that Baumé, e. g., 33° Bé. In other cases, where the solutions which I employed ran between 30 and 40° Bé., corresponding brush solutions never in practice run higher than 12° or 15° Bé.

As to the attrition material employed, I can obtain good felts by utilizing concentrated carrots with abrasive materials, but because of the waste incident to the use of these abrasives, as translated into cost per pound of the raw fur, I do not consider this the best practice. It is much more commercially satisfactory to employ an at-

trition material which is non-abrasive, such as rubber, plastic or resinous materials to which I have referred and of these latter materials the best results have been obtained by using an attrition material, the specific gravity of which runs under 2 and may, to advantage, approximate the specific gravity of the pelts. The advantage of this is that the attrition material tends to more evenly distribute itself throughout the fur during the tumbling operation and with this low specific gravity, a better distribution of relatively light material is obtained with consequent wider distribution of a larger superficial area for the carrying of the carroting solution, without the superimposition upon the fur of too heavy a mass of carrier material. This latter consideration minimizes damage to the fur fibers and consequently renders the loss of fur negligible.

Having thus fully described the invention, what I claim as new and desire to secure by Letters Patent is:

1. The process of carroting fur on the pelt, which comprises: admixing a highly active concentrated chemical carroting solution, in sufficient amount to carrot the fur when rubbed against the fur fibers, with a sufficient amount of pieces of substantially acid-proof and substantially non-absorbent solid attrition material, to carry the chemical carroting solution to the exclusion of free flowing liquid, thereafter tumbling the thus treated pieces of attrition material with the pelts to rub the carroting solution against the fur fibers thereof, and thereafter separating the attrition material from the pelts.
2. The process of carroting fur on the pelt, which comprises: admixing a highly active concentrated chemical carroting solution, in sufficient amount to carrot the fur when rubbed against the fur fibers, with a sufficient amount of pieces of substantially acid-proof and substantially non-absorbent solid attrition material to carry the chemical carroting solution to the exclusion of free flowing liquid, thereafter tumbling the thus treated pieces of attrition material with the pelts to rub the carroting solution against the fur fibers thereof, thereafter separating the attrition material from the pelts, and subjecting the thus carotted fur on the pelts to the action of moving heated air.
3. The process of carroting fur on the pelt, which comprises: admixing a highly active concentrated chemical carroting solution, in sufficient amount to carrot the fur when rubbed against the fur fibers, with a sufficient amount of pieces of substantially acid-proof and substantially non-absorbent solid attrition material of a specific gravity less than 2 to carry the chemical carroting solution to the exclusion of free flowing liquid, thereafter tumbling the thus treated pieces of attrition material with the pelts to rub the carroting solution against the fur fibers thereof, and thereafter separating the attrition material from the pelts.
4. The process of carroting fur on the pelt, which comprises: admixing a highly active concentrated chemical carroting solution, in sufficient amount to carrot the fur when rubbed against the fur fibers, with a sufficient amount of pieces of non-abrasive substantially acid-proof and substantially non-absorbent solid attrition material of a specific gravity less than 2 to carry the chemical carroting solution to the exclusion of free flowing liquid, thereafter tumbling the thus treated pieces of attrition material with the pelts to rub the carroting solution against the

fur fibers thereof, and thereafter separating the attrition material from the pelts.

5. The process of carrottting fur on the pelt, which comprises: admixing a highly active concentrated chemical carrottting solution, in sufficient amount to carrot the fur when rubbed against the fur fibers, with a sufficient amount of pieces of substantially acid-proof and substantially non-absorbent solid attrition material to carry the chemical carrottting solution to the exclusion of free flowing liquid, covering the flesh sides of the pelts prior to carrottting the fur, thereafter tumbling the thus treated pieces of attrition material with the pelts, while the flesh sides thereof are covered, to rub the carrottting solution against the fur fibers thereof, and thereafter separating the attrition material from the pelts.

6. The process of carrottting fur on the pelt, which comprises: admixing a highly active concentrated chemical carrottting solution, in sufficient amount to carrot the fur when rubbed against the fur fibers, with a sufficient amount of pieces of substantially acid-proof and substantially non-absorbent solid attrition material to carry the chemical carrottting solution to the exclusion of free flowing liquid, folding the pelts prior to carrottting the fur so that the lateral halves of each pelt mutually overlie and cover the flesh sides of one another, thereafter tumbling the thus treated pieces of attrition mate-

rial with the folded pelts to rub the carrottting solution against the fur fibers thereof, and thereafter separating the attrition material from the pelts.

5 7. The process of carrottting fur on the pelt which comprises: tumbling the pelts with a relatively large bulk of pieces of substantially acid proof attrition material substantially free from abrasive properties and dust and carrying a substantially imperceptible coating of adsorbed highly active concentrated carrottting solution, and thereafter separating the attrition material from the pelts.

8. The process of carrottting fur on the pelt, 15 which comprises: admixing a highly active concentrated chemical carrottting solution containing at least one acid selected from the group consisting of nitric and sulphuric acid together with hydrogen peroxide, in sufficient amount to carrot 20 the fur when rubbed against the fur fibers, with a sufficient amount of pieces of substantially acid-proof and substantially non-absorbent solid attrition material to carry the chemical carrottting solution to the exclusion of free flowing liquid, 25 thereafter tumbling the thus treated pieces of attrition material with the pelts to rub the carrottting solution against the fur fibers thereof, and thereafter separating the attrition material from the pelts.

30

JACK D. SARTAKOFF.